

# UNITED STATES PATENT OFFICE.

HOWARD F. WEISS, OF MADISON, WISCONSIN, ASSIGNOR TO C. F. BURGESS LABORATORIES, OF MADISON, WISCONSIN, A CORPORATION OF WISCONSIN.

## FIREPROOFING OF WOOD.

1,346,287.

Specification of Letters Patent. Patented July 13, 1920.

No Drawing.

Application filed August 17, 1918. Serial No. 250,328.

*To all whom it may concern:*

Be it known that I, HOWARD F. WEISS, a citizen of the United States, residing at Madison, in the county of Dane, State of Wisconsin, have invented certain new and useful Improvements in Fireproofing of Wood; and I do hereby declare the following to be a full, clear, and exact description of the invention, such as will enable others skilled in the art to which it appertains to make and use the same.

In the fire-proofing of wood, to which the present invention relates, it has heretofore been customary to treat the wood, especially when in the form of shingles, in one or the other of two ways, viz: either by dipping the wood into, or painting it with, a liquid fire-proofing composition, or by injecting a water soluble fire-resisting chemical of some character into the wood. Both of these treatments, however, are superficial only, and produce merely temporary results, so that their effectiveness gradually becomes impaired, and they must, in consequence, be repeated from time to time. Thus, in the first instance, the paint wears off; and furthermore, if the painted surface is once punctured by the fire, the wood on the inside is fully combustible. In the second instance, the chemicals usually employed, such as ammonium phosphate, ammonium sulfate, etc., are soluble in water, and it becomes necessary, therefore, to coat the surface of the wood with a substance which will prevent them from washing out. Here again, the treatment is temporary only, as the outside protective coating wears off in time and, unless renewed, leaves the soluble chemicals free to be washed out.

It has been proposed to overcome the defects of the aforesaid methods by injecting into the wood two water soluble chemicals, for example zinc chlorid and borax, which are capable of combining and forming a salt (zinc borate) which is insoluble in water. The two chemicals are applied separately, however, and the wood is dried after each impregnation, so that while the actual results obtained by or from this method have proven satisfactory, the method itself is tedious and extremely costly.

It is the object of the present invention to provide a method of fireproofing wood, primarily in shingle form, which, while possessing all of the advantages of the two-

chemical treatment just described, yet involves the impregnation of the wood with a single chemical only, so that the cost of the treatment is greatly reduced as compared with the former procedure, and the wood so treated retains its fire-retardant and non-combustible properties for indefinite periods of time, even when exposed to the weather, or to running water.

According to the invention, there is injected into the wood a chemical which is initially and under ordinary conditions soluble in water, but which, after it has been forced into the wood, will change over into an insoluble chemical upon drying. Barium sulfid, either crude or refined, has proven eminently satisfactory for this purpose; and in carrying the invention into practice, a solution of that chemical is forced under pressure into the wood in much the same manner that wood is creosoted, after which the wood is removed from the cylinder impregnated with the barium sulfid solution and allowed to dry in the air, the barium combining with carbon dioxid in the atmosphere and changing into insoluble barium carbonate, while the sulfur combines with hydrogen to form hydrogen sulfid and eventually passes off in the atmosphere. In this way, the wood is ultimately filled with an insoluble chemical, barium carbonate, which renders it permanently fire-resistant to a high degree and practically non-combustible. Western red cedar shingles treated according to this method have been subjected to the flame of a Bunsen burner for five minutes at a temperature of 1600° F., no ignition whatever taking place, but the shingles merely becoming converted into charcoal; whereas untreated shingles and the so-called "asphalt" shingles covered with crushed stone or slate, burned violently under the same conditions, and were completely destroyed.

The change of the barium into barium carbonate can be greatly hastened and facilitated by drying the wood in an atmosphere containing more carbon dioxid. This step may be effectively carried out by running the impregnated wood into a kiln, and passing carbon dioxid gas thereinto with the ordinary air, considerable quantities of the gas being readily obtainable from flue gases. Experiments have shown that while a certain amount of the barium in the wood

will go over to the insoluble carbonate when the wood is exposed to the air, nevertheless, larger amounts and better results are secured if the drying is done in an atmosphere containing more carbon dioxid than is present ordinarily in the atmosphere.

I claim as my invention:

1. A one-solution method of fireproofing wood, which comprises impregnating the wood with an aqueous solution of a soluble barium sulfid, and then converting said soluble barium compound into insoluble barium carbonate by treatment with gaseous carbon dioxid, whereby the sulfur of the said barium sulfid is expelled as hydrogen sulfid and the said insoluble barium carbonate is formed within the body of the wood, extending inwardly from the periphery of the same.
2. The method of fireproofing wood, which comprises impregnating the wood with an aqueous solution of a soluble alkaline earth compound, and then, while

drying the wood, converting said soluble compound into an insoluble compound by treatment with a suitable gaseous precipitating agent, whereby the said insoluble compound is formed within the body of the wood, extending inwardly from the periphery of the same.

30

3. The method of fireproofing wood, which comprises impregnating the wood with an aqueous solution of a soluble alkaline earth sulfid, and then, while drying the wood, converting said soluble compound into an insoluble alkaline earth carbonate by treatment with gaseous carbon dioxid.

4. The method of fireproofing wood, which comprises impregnating the wood with an aqueous solution of a soluble barium sulfid, and then, while drying the wood, converting said soluble compound into insoluble barium carbonate by treatment with gaseous carbon dioxid.

In testimony whereof I affix my signature.

HOWARD F. WEISS.